

# United States Patent [19]

Hammerstein et al.

[11] 3,804,629

[45] Apr. 16, 1974

[54] **PROCESS FOR THE PRODUCTION OF A STAIN-RESISTANT PHOTOGRAPHIC SILVER HALIDE EMULSION**

[75] Inventors: **Hanns Hammerstein**, Hamburg; **Helmut Reuss**, Leverkusen; **Erik Moisar**, Cologne, all of Germany

[73] Assignee: **Agfa-Gevaert Aktiengesellschaft**, Leverkusen, Germany

[22] Filed: Sept. 5, 1972

[21] Appl. No.: 286,291

[30] **Foreign Application Priority Data**

Sept. 3, 1971 Germany..... 2144127

[52] U.S. Cl. .... 96/94 R, 96/110

[51] Int. Cl. .... G03c 1/02, G03c 1/72

[58] Field of Search..... 96/110, 94

[56] **References Cited**

UNITED STATES PATENTS

3,600,180 8/1971 Judd et al. .... 96/94 R

*Primary Examiner*—Norman G. Torchin

*Assistant Examiner*—Alfonso T. Suro Pico

*Attorney, Agent, or Firm*—Connolly and Hutz

[57] **ABSTRACT**

The stability of silver halide emulsion layers against the deleterious effect of dust in particular metal dust is improved by adding to the physically ripened and washed emulsion before chemical ripening a silver chloride emulsion or by precipitating silver chloride on to the physically ripened and washed silver halide emulsion.

**3 Claims, No Drawings**

PROCESS FOR THE PRODUCTION OF A  
STAIN-RESISTANT PHOTOGRAPHIC SILVER  
HALIDE EMULSION

The invention relates to a method for decreasing the formation of small stains caused by the presence of heavy metals and/or their compounds or other contaminating substances in photographic silver halide emulsions, auxiliary layers and supports for photographic silver halide emulsions.

It is known that cleanliness is extremely important in the manufacture of light-sensitive photographic materials. Photographically active dust such as abrasion dust from metal contaminates the light-sensitive silver halide emulsion layer in spite of all precautions. The metal particles or their compounds or other photographically active substances dissolve in the photographic layers, auxiliary layers or supports with varying degrees of rapidity. The dissolved products diffuse in the layers and are liable to cause considerable harm to the photographic properties, e.g. by exerting a sensitizing or desensitizing effect. The well-known black or white patchiness is then found in the light-sensitive photographic materials after they have been processed in photographic baths in the usual manner.

A similar harmful effect may also be caused by impurities e.g. in the raw material used for the production of the paper support. In that case, black or white patchiness is found in the material after development, especially if the material is stored under conditions of elevated temperature and moisture.

Various additives have been described for preventing this effect. These additives are incorporated either in the emulsion or in adjacent layers. Most of these substances, however, produce only a slight effect whilst others become sufficiently effective only at high concentrations at which they often give rise to other harmful side effects.

It is an object of this invention to modify the process for producing the photographic silver halide emulsion so that patchiness due to the presence of dust and heavy metal particles will not occur.

A process for the production of a photographic silver halide emulsion comprising the steps of precipitation of the silver halide in the presence of a protective colloid, physical ripening, washing of the ripened emulsion to remove the soluble salts and chemical ripening has now been found in which a gelatin emulsion containing essentially only silver chloride is added to the physically ripened and washed emulsion before it is chemically ripened, or the silver chloride which is to be added is produced in the physically ripened and washed silver halide emulsion by precipitation by the addition of alkali metal chloride and silver nitrate solutions.

The method according to the invention results in the formation of silver chloride hillocks on the silver halide grains of the original emulsion. These hillocks surprisingly produce excellent resistance to the formation of stains by particles of dirt. These silver chloride hillocks on the particles of the original silver halide emulsions, which is preferably a silver bromide emulsion, are clearly visible under an electron microscope.

The concentration of silver chloride produced in the original silver halide emulsion either by the addition of a silver chloride emulsion or by precipitation may vary within wide limits. The optimum quantity can be determined by tests well known in the art. Quantities of from

2 to 10 mol % of silver chloride, based on the total quantity of silver halide in the physically ripened and washed emulsion have generally been found to effect sufficient stabilization for practical purposes.

5 It is preferable to use an excess of chloride ions for producing the silver chloride hillocks. This excess should preferably be from 1.2 to 2 times to required equimolar quantity of chloride ions.

The production of silver halide emulsions modified in 10 accordance with the invention is otherwise carried out by the usual process which comprises the following steps:

1. Precipitation of the silver halides in the presence of a protective colloid and physical ripening;

15 2. Removal of the excess water-soluble salts formed in the process of precipitation by washing the ripened emulsion; and

20 3. Chemical ripening of the washed emulsion to provide the desired photographic properties, in particular the desired sensitivity.

The silver halides used for the emulsion which is to be stabilized may be silver chloride, silver bromide or mixtures of these if derived with a silver iodide content of up to 10 %. The silver halides are dispersed in the 25 usual hydrophilic binders, e.g. in proteins, preferably gelatin, carboxymethyl-cellulose, polyvinyl alcohol, polyvinyl pyrrolidone or alginic acid and its derivatives such as salts, esters or amides.

After the treatment with silver chloride in accordance 30 with the invention, the emulsions may be chemically ripened in the usual manner and treated with the usual additives. The emulsion may be optically sensitized with cyanines rhodacyanines or merocyanines, e.g. as described in "The Cyanine Dyes and related 35 Compounds" by F. M. HAMER, published by Interscience Publishers (1964).

The emulsions may be chemically sensitized in the usual manner, e.g. with reducing agents such as tin(II) salts, polyamines such as diethyltriamine or sulfur compounds 40 as described in U.S. Pat. specification No. 1,574,944. Salts of noble metals such as ruthenium, rhodium, palladium, iridium, platinum or gold may also be added as chemical sensitizers, as described in the publication by R. KOSLOWSKY in Z. Wiss. Phot. 46, 65 - 72 (1951). The emulsions may also contain polyalkylene oxides as chemical sensitizers and in particular polyethylene oxides and derivatives thereof.

The emulsions may be stabilized against spontaneous 50 fogging by the addition of the usual stabilizers such as organic mercury compounds or mercury salts, e.g. mercury triazole compounds, simple mercury salts or mercury double salts. Other useful stabilizers are in particular azaindenes, e.g. tetra- or pentaazaindenes and particularly those which are hydroxyl substituted or amino substituted, as described in the publication by BIRR in Z. Wiss. Phot. 47, 2 - 58 (1952). Heterocyclic mercapto compounds such as 1-phenyl-5-mercaptopentetrazole, quaternary benzothiazole derivatives and benzotriazoles may also be used.

55 The emulsion is hardened in the usual manner, e.g. with aldehydes such as formaldehyde, dialdehydes or halo substituted aldehydes which contain a carboxyl group, e.g. mucochloric acid or mucobromic acid, or diketones or sulfonic acid esters such as methanesulfonic acid esters.

The emulsions prepared in accordance with the invention may be used for various photographic materi-

als. They are particularly suitable for silver halide emulsion layers used for photographic copying materials mounted on a paper support but they may also be used for X-ray films, unsensitized emulsions, orthochromatically or panchromatically sensitized emulsions or emulsions which are sensitive to the infra-red region of the spectrum. The emulsions may be used in materials for the silver salt diffusion process, in color photographic materials and also in photographic materials for the silver dye bleaching process.

#### EXAMPLE 1

A silver bromide emulsion containing 14 mols % of silver chloride and 1 mol % of silver iodide is prepared in the usual manner by precipitation in the presence of gelatin.

The emulsion is flocculated after physical ripening and the soluble salts resulting from precipitation are removed by washing with water. The silver halide is then melted at pH 5.5 with the addition of gelatin and water. The emulsion then contains 55 g of silver halide per kg and 220 g of gelatin per kg. It is then ripened to the required sensitivity at 53°C.

In addition, the following additives are introduced into the casting solution:

10 ml of a 0.1 % aqueous solution of optical sensitizer of the following formula:



10 ml of a 1 % aqueous solution of a 2-mercaptopro-4-keto-3,4-dihydro-pyrimidine of the following formula as stabilizer:



20 ml of a 5 % aqueous solution of saponin and 0.75 ml of a 30 % aqueous solution of formaldehyde.

The emulsion is applied to a baryta-coated paper support to which a layer of gelatin containing iron dust has been applied to test the effectiveness of the process according to the invention.

The emulsion is uniformly exposed and developed in a developer of the following composition:

|                                       |                        |
|---------------------------------------|------------------------|
| p-methylaminophenol                   |                        |
| Na <sub>2</sub> SO <sub>3</sub> sicc. | 13 g                   |
| hydroquinone                          | 3 g                    |
| soda sicc.                            | 26 g                   |
| KBr                                   | 1 g per litre of water |

The sample obtained after processing is uniformly black. It has numerous white patches which can be attributed to the harmful effect of the iron dust.

In another test, an emulsion is prepared by the same method except that, after washing and before chemical ripening, 20 ml of a 10 % aqueous sodium chloride so-

lution and 83 ml of a 5 % aqueous silver nitrate solution are added. When precipitation takes place, hillocks of silver chloride are formed on the grains of the original emulsion. The quantity of silver chloride produced by precipitation is 8.3 mols % of silver chloride based on the amount of silver halide in the original emulsion. The emulsion is then chemically ripened and processed as described above.

The developed and fixed sample is practically free from stains. In the case of the emulsion prepared according to the invention, practically no white stains are formed even if the sample has been stored in an air conditioning cupboard at 60°C and 40 % atmospheric humidity for 2 days before processing. In the comparison emulsion the formation of stains is increased under these conditions.

#### EXAMPLE 2

A silver bromide emulsion containing 4.8 mols % of silver chloride and 1.5 mols % of silver iodide is prepared in the usual manner by precipitation in the presence of gelatin as protective colloid.

It is physically ripened and the emulsion is flocculated and the soluble salts are removed by washing. The silver halide is then redispersed by the addition of gelatin and water at pH 5.5. The emulsion then contains 55 g of silver halide and 160 g of gelatin per kg.

The emulsion is then divided into two portions. 4 ml of a 10 % sodium chloride solution and 17 ml of a 5 % aqueous silver nitrate solution are added to one portion. The quantity of silver chloride produced, which forms hillocks on the grains of the original silver bromide emulsion, is 1.7 mols %, based on the amount of original emulsion.

Both portions are then chemically sensitized to the required sensitivity under the same conditions at 49°C. Saponin and formaldehyde are then added as in Example 1 and in addition 5.3 ml of a 1 % methanolic solution of 1-phenyl-5-mercaptopentetrazole as stabilizer.

The material is processed in the same way as described in Example 1.

Examination of the resulting sample shows that the formation of white stains has again been practically completely suppressed by the process according to the invention while the comparison sample has numerous white stains.

#### EXAMPLE 3

The procedure is the same as that described in Example 1, but instead of adding sodium chloride solution and silver nitrate solution to the physically ripened and washed emulsion, a previously prepared silver chloride gelatin emulsion is added.

The subsequent treatment is the same as described in Example 1. Examination of the sample shows equally good results to those obtained in Example 1.

Equally effective stabilization and prevention of the formation of white stains is achieved if instead of the pure silver chloride emulsion, a silver chloride emulsion which contains 3 mols % of silver bromide and 0.05 mols % of silver iodide is added to physically ripened and washed silver bromide emulsion.

The gelatin content in the silver chloride emulsions described above is 180 g/kg.

We claim:

1. In a process for the production of photographic silver halide emulsions by precipitation of the silver ha-

lides in the presence of protective colloids, physical ripening, washing and chemical ripening, the improvement according to which a silver chloride emulsion is added to the physically ripened and washed emulsion before chemical ripening or silver chloride is produced in the washed emulsion by precipitation by the addition of an aqueous alkali metal chloride and aqueous silver salt solution.

2. The process of claim 1, wherein from 1.2 to 2

times the equimolar quantity of chloride ions is present when the silver chloride emulsion is added or the silver chloride is formed by precipitation.

3. The process of claim 1, wherein the amount of silver chloride introduced by the addition of silver chloride or by precipitation in the washed emulsion is from 2 to 10 mols %, based on the silver halide of the original silver halide emulsion.

\* \* \* \* \*

10

15

20

25

30

35

40

45

50

55

60

65